

A. H. EMERY.

PROCESS OF REGULATING INITIAL STRAINS IN ROLLING STRUCTURAL MATERIAL.

APPLICATION FILED MAY 26, 1908.

939,676.

Patented Nov. 9, 1909.

Fig. 3.



Fig. 2.



Fig. 1.



Witnesses

J. M. Winkler  
E. B. Quist

Inventor

Albert H. Emery.  
by Knight Bros. Attorneys.

# UNITED STATES PATENT OFFICE.

ALBERT H. EMERY, OF STAMFORD, CONNECTICUT

## PROCESS OF REGULATING INITIAL STRAINS IN ROLLING STRUCTURAL MATERIAL.

939,676.

Specification of Letters Patent.

Patented Nov. 9, 1909.

Application filed May 26, 1908. Serial No. 435,115.

To all whom it may concern:

Be it known that I, ALBERT H. EMERY, a citizen of the United States, residing at Stamford, in the county of Fairfield and 5 State of Connecticut, have invented a certain new and useful Process of Regulating Initial Strains in Rolling Structural Material, of which the following is a specification, reference being had to the accompanying drawing, in which—

Figures 1, 2 and 3 are transverse sectional views of an I-beam, an H-beam and a channel-beam respectively, with figures showing their several dimensions and proportions, as 15 commonly rolled by large American rolling mills.

My invention has for its object the control of the initial strains developed in rolled structural material during the process of 20 rolling and cooling and is especially applicable to forms where some of the parts of a cross section are much thicker than other parts. In rolling I-beams, angles and other flanged members, strains are set up by both 25 the rolling and the cooling. If the parts were rolled of equal thickness, and all parts of the member of one temperature at the time the rolling was completed then the strains would remain in kind and largely 30 in degree what they were at the end of the last pass between the rolls. But in most cases there is a large relative difference between the thickness of the thicker and thinner parts of the member—and the thicker 35 part is likely to be much hotter than the thinner part when the rolling is completed. Should the rolling have been done in such a way that the member leaves the rolls without initial strains, then this unequal heat of 40 the thicker and thin parts will set up initial strains as the cooling proceeds, and these initial strains in the ordinary cooled I-beam are often very great, and usually so great in angles and I-beams as to be very objectionable; the thin parts of the cooled members being usually under large strains of compression and the thicker parts under strains 45 of tension. In the case of I-beams the flanges are usually thicker and hotter than the webs which join them and their unequal heat causes the flanges to contract more in cooling than do the webs, and this unequal contracting sets up strains of tension in the thicker parts and compression in the thinner parts of the member. To avoid this it is 50 desirable to have all parts of the member of

a uniform heat at time of last pass between the rolls, but this is not easy to do. We may use water or other cooling mediums to spray the members and help to cool the thicker parts as the work proceeds and even then we shall usually find so great difference of temperatures of the thicker and thinner parts that if rolled free from strains, strains will be set up in the cooling so that it is better to 55 set up initial strains in the members during the last part of the rolling by reducing the thicker part proportionally more than we do the thinner parts, and this extra reduction will cause at the completion of the rolling 60 compression in the thicker part and tension in the thinner part of the member and these strains being the reverse of those which would be produced by cooling, they may be made to largely neutralize each other, or if 65 we choose we may even carry this process so far as to leave the cooled member with compression on the thicker part and tension on the thinner parts, if in any case such a condition were desired.

The cooling of the thicker part of the metal by spraying or otherwise, as the work proceeds, to bring the temperature down toward that of the thinner parts, before the rolling is completed, has the effect, usually, 70 of causing the latter part of the rolling to be done at a lower temperature than that at which it would otherwise be done when no attention is paid to this matter, and this rolling at the lower heat, makes the metal 75 stronger and tougher than it would be if rolled at a higher heat. The excess of the reduction of the thicker parts over that of the thinner parts during the last pass, or during the latter part of the rolling, may 80 result from a certain reduction in the thicker parts with no reduction, at that time, in the thinner parts, or from a reduction of the thicker parts, together with such a reduction of less degree in the thinner parts as will 85 give the desired excess of reduction in the thicker.

To explain my invention more in detail, I will refer to one of its numerous applications, to wit: the rolling of I-beams and particularly, heavily flanged I-beams see Fig. 1. These are best rolled by making use of one pair of horizontal rolls to form the web and inner faces of the flanges, and a pair of rolls in the same plane, but with vertical 90 axes, to roll the outer faces of the flanges or heads of the beam, because such a system

of rolls facilitates setting up the vertical rolls relatively to or independently of the setting up of the horizontal rolls, preparatory to the last pass of the beam between the rolls, or the latter part of the rolling operation for the purpose of reducing the heads or thicker portions of the beam, without reduction of the web, or with proportionately less reduction of the web.

10 Should the final rolling be accomplished by a pass between single pairs of rolls only, it would be more difficult to properly do the work, because the fixed form of the rolls for the final pass cannot be changed to suit the changing temperatures of the members, and consequently, it will be necessary to control the heat more closely, to bring about the desired result, than when using the system of rolls first mentioned, or else have 15 several pairs of rolls or a series of slightly varying grooves in one pair of rolls through either of which sets of grooves the last pass may be made at will, the grooves used depending upon the relative temperatures of 20 the thick and thin parts of the member being rolled.

Having thus described my invention, what I claim as new therein, and desire to secure by Letters Patent is:—

30 1. The process of regulating the initial strains in rolled structural material which consists in developing by rolling, while rolling from a heated blank, strains that partly neutralize the strains that would otherwise 35 be set up in the member when cooled and thus decrease injurious strains when the member is cooled.

2. The process of regulating the initial strains in rolled structural material which 40 consists in developing during rolling, while rolling from a heated blank, strains of compression in the thicker part and tension in the thinner part so that said strains tend to counteract or avoid injurious strains 45 when the member is cooled.

3. The process of regulating the initial strains in rolled structural material which 50 consists in developing during rolling, while rolling from a heated blank, strains of compression in the thicker part and tension in the thinner part, of such magnitude at the completion of the rolling, that said strains

largely neutralize the strains that would otherwise result from unequal contraction in cooling.

55

4. The process of regulating initial strains in rolling structural material from heated blanks which consists in regulating the rolling during the last pass between the rolls so that the percentage reduction of the thick 60 part of the member is sufficiently greater than that of the thin part, as to cause, strains of compression in the thick part and tension in the thin part which strains will be partly or wholly relieved in cooling.

65

5. The process of regulating the initial strains in rolled structural material which consists in artificially cooling the thicker parts of the member while rolling, and in developing, in the final rolling, strains of 70 compression in the thicker part and tension in the thinner part so that said strains tend to counteract or avoid injurious strains when the member is cooled.

6. The process of regulating the initial strains in rolled structural material which consists in artificially cooling the thicker parts of the member while rolling, and in developing, in the final rolling, strains of 75 compression in the thicker part and tension 80 in the thinner part, of such magnitude at the completion of the rolling, that said strains neutralize the strains that would otherwise result from unequal contraction in cooling.

85

7. The process of regulating the initial strains in rolled structural material which consists in artificially cooling the thicker part of the member and in regulating the 90 rolling during the last pass between the rolls so that the percentage reduction of the thick part of the member is sufficiently greater than that of the thin part, as to cause strains of compression in the thick part and tension in the thin part, which 95 strains will be partly or wholly relieved in cooling.

The foregoing specification signed at Washington, District of Columbia, this 22nd day of May, 1908.

ALBERT H. EMERY.

In presence of—

HERVEY S. KNIGHT,  
EDWIN S. CLARKSON.